

## UNITED STATES PATENT OFFICE.

WILLIAM H. BASSETT, JR., OF ANSONIA, CONNECTICUT, ASSIGNOR TO THE AMERICAN BRASS COMPANY, OF WATERBURY, CONNECTICUT, A CORPORATION OF CONNECTICUT.

## WROUGHT-METAL ARTICLE.

No Drawing.

Application filed January 28, 1926. Serial No. 84,508.

My invention relates to an improvement in wrought metal articles and consists of a wrought metal article composed of a copperous alloy hereinafter described containing

5 tin and aluminum within certain ranges. I have discovered that this alloy has good electrical conductivity, very high strength, excellent resistance to fatigue, is extremely ductile, exceedingly malleable, and has very 10 high resistance to atmospheric corrosion and better resistance to the action of corrosive substances, such as acids and alkalies, and greater electrical conductivity than has previously been obtained with alloys of copper, 15 tin and silicon, or alloys of copper, zinc and nickel hitherto employed where the following properties were requisite, strength, malleability, ductility, electrical conductivity, resistance to fatigue and resistance to corrosion.

The alloy of the invention was developed by a series of experiments in which I found that while the aluminum copper alloys had the requisite strength, they were apt to be 25 "slivery", difficult to manufacture, and were of low electrical conductivity. The copper-tin alloys while having better electrical conductivity, either could not be hot rolled or became brittle when the requisite strength 30 was obtained by cold working. The improved alloy of the invention has given the desired results while avoiding the difficulties encountered in the alloys previously used. It is comprised chiefly of copper, aluminum 35 and tin.

I have discovered that an alloy of these metals can be easily hot rolled and forged and cold rolled or cold drawn, and that when cold drawn has high ductility so that it 40 can be bent without breaking. It can also be extruded and hot pressed. It is a good conductor of electricity and highly resistant to corrosion and of high tensile strength. It also has high resistance to fatigue when 45 wrought. It resists atmospheric corrosion to a high degree and is not easily attacked by acids and alkalies. It does not age so as to become brittle and is of relatively low manufacturing cost. So far as I know, no alloy

of these metals has ever been put to any 50 practical use and the alloy specifically set forth has never been known or described before my invention thereof.

The chief objects of my invention are to provide a wrought article composed of an 55 alloy having these characteristics.

My invention also has for its object to provide wrought metal articles which are particularly adapted for electric railway line material and high strength cables, or cable 60 elements, contact trolley wires, telephone or telegraph wires, electric railway line hardware and the like.

The alloy used by me is composed essentially of copper, tin and aluminum. In its 65 preferred form the proportions are 95.5% copper, 2% tin and 2.5% aluminum. Such an alloy has the advantages and characteristics above referred to and can be used for the purposes specified. The proportions can 70 be varied somewhat but when 98.5% copper, 1% tin and 0.5% aluminum are used the tensile strength is materially reduced, and when 91% copper, 5% tin and 4% aluminum are used the workability is materially reduced, and in embodying my invention I do 75 not exceed these limits.

In producing the alloy I bring the copper to a molten condition at pouring temperature and then introduce the tin and later the 80 aluminum, stirring meanwhile so as to produce a uniform mixture. In order to attain the best results, high purity metals should be used and the oxides kept as low as possible. In forming the alloy I keep a layer 85 of charcoal on the surface of the molten material.

Wire composed of the described alloy is an important embodiment of my invention. Such wire is made by the usual methods, 90 such as extruding or hot rolling ingots into rods and cold drawing the rods into wire. My wire has a tensile strength of over 100,000 pounds to the square inch but notwithstanding is of high ductility so that it can 95 be bent around a wire of its own diameter without breaking, and will withstand other tests usually applied to ductile material.

As will be evident to those skilled in the art, my invention permits of various modifications without departing from the spirit thereof or the scope of the appended claims.

5. What I claim is:

1. A new wrought metal article composed of an alloy consisting essentially of copper and tin with aluminum, approximately in the proportions copper 95.5%, tin 2%, aluminum 2.5%, the aluminum being in excess of the tin.
10. 2. A cold drawn wire composed of an alloy consisting essentially of copper and tin with aluminum in the proportions copper 98.5% to 91%, tin 1% to 5%, aluminum 0.5% to 4%.
15. 3. A metallic wire made by hot rolling and cold drawing of an alloy composed essentially of 98.5% to 91% copper, and 1% to 5% tin, with the addition of 0.5% to

4% aluminum as a deoxidizing and strengthening agent.

4. A metallic wire adapted to be used individually or in the construction of cables for use in transmission lines, messengers, contact wires, telephone lines, telegraph lines, guys, cross spans, stays, or hangers, said metallic wire being composed essentially of 98.5% to 91% copper, and 1% to 5% of tin, with 0.5% to 4% aluminum. 25

5. A metallic wire composed of an alloy consisting essentially of copper and tin with aluminum in approximately the proportions copper 95.5%, tin 2%, aluminum 2.5%, the aluminum being in excess of the tin. 30

In testimony whereof, I have signed my name to this specification this twenty-fifth day of January, 1926.

WILLIAM H. BASSETT, JR.